

## UNITED STATES PATENT OFFICE

JOHN A. GANN, OF MIDLAND, MICHIGAN, ASSIGNOR TO THE DOW CHEMICAL COMPANY, OF MIDLAND, MICHIGAN, A CORPORATION OF MICHIGAN

## MAGNESIUM-MANGANESE-ZINC ALLOYS

No Drawing.

Application filed November 20, 1930. Serial No. 497,077.

The present invention relates to ternary magnesium alloys in which magnesium is the predominant metal, and specifically to magnesium-manganese-zinc alloys.

5 Magnesium is the lightest of the engineering metals. This property in connection with good tensile strength makes it a highly desirable metal where reduction in weight is a prime consideration as in air and land vehicles. Accordingly, numerous efforts have been made to produce suitable alloys for such uses. The addition of zinc to magnesium in order to make a binary light metal alloy has been heretofore described in U. S. Patent No. 982,022 to Rübel dated Jan. 17, 1911, the stated proportions of the zinc being not less than 1 per cent nor more than 6 per cent, and in a more recent U. S. Patent No. 1,377,874 to William R. Veazey dated May 10, 1921, a binary alloy is disclosed consisting of magnesium to which manganese has been added. However, I have discovered by carrying out many extensive investigations and numerous carefully conducted tests both 15 of a scientific character and under conditions of practical use that a ternary alloy containing all three of the elements magnesium, manganese, and zinc will largely overcome or mitigate the drawbacks of each of the above 20 noted binary alloys, and at the same time produce an alloy having substantially all of their good properties.

Accordingly, among the objects of the present invention is the production of ternary 35 alloys containing magnesium, manganese, and zinc, such alloys having high corrosion resistance and superior mechanical properties. Other objects and advantages will appear as the description proceeds.

40 The invention, then, consists of the new product consisting of a ternary alloy of the metals magnesium, manganese, and zinc as hereinafter fully described and particularly set forth in the claims. The following description, it will be understood, thus sets forth 45 but several of various ways in which the invention may be carried out.

The new ternary magnesium-manganese-zinc alloys have very good properties when 50 in the form of cast articles and moreover

such alloys can be heat treated and/or readily worked as by rolling, forging, or extruding to form articles having still better properties. The general features of these new ternary alloys can be best set forth by comparing the properties of one specific magnesium-manganese-zinc alloy with the like properties of a binary magnesium-manganese alloy and a binary magnesium-zinc alloy having the same percentages of manganese and zinc respectively as contained in the ternary alloy. The following table gives the properties of these alloys in the "as cast" state.

Properties of sand cast magnesium alloys

|                            | Mg+Zn<br>(3%) | Mg+Mn<br>(1.4%) | Mg+Mn<br>(1.4%) +<br>Zn (3%) | 65 |
|----------------------------|---------------|-----------------|------------------------------|----|
| Tensile strength #/sq. in. | 26000         | 18000           | 26000                        |    |
| Yield point #/sq. in.      | 5000          | 3500            | 5000                         | 70 |
| Per cent elongation        | 12            | 8               | 11                           |    |
| Brinell hardness           | 37            | 34              | 37                           |    |
| Impact ft. lbs.            | 11            | 10              | 12                           |    |

Referring to the table, it is noted that the ternary magnesium-manganese-zinc alloy is 75 superior in every way to the corresponding binary magnesium-manganese alloy. Its mechanical properties likewise very closely approximate those of the corresponding binary magnesium-zinc alloy. It is thus to be seen 80 that the addition of zinc to a binary magnesium-manganese alloy makes a very marked improvement in its mechanical properties, and accordingly, the new ternary alloy can be considered as an improvement over the binary magnesium-manganese alloy. The corrosion resistance of the ternary magnesium-manganese-zinc alloy further is far superior to that of the binary magnesium-zinc alloy 85 and very closely approaches that of the binary magnesium-manganese alloy which at the present time exhibits the best corrosion resistance of any magnesium alloy being produced. To summarize the above, the new ternary magnesium-manganese-zinc alloys have 90 a corrosion resistance closely approaching that of the highly corrosion resistant binary magnesium-manganese alloys, and at the same time have mechanical properties substantially equivalent to binary magnesium- 95

100

zinc alloys which are among the strongest of the binary magnesium alloys. These new ternary alloys accordingly are exceptionally well suited to usages where both strength and corrosion resistance are essential.

5 The improved ternary magnesium-manganese-zinc alloys can be formed from their components, for instance by melting a quantity of magnesium and adding thereto the metals manganese and zinc or by adding to 10 the molten magnesium a manganese-zinc alloy. Another satisfactory method of adding manganese to the metal consists, as described in the above noted U. S. Patent No. 1,377,374 to W. R. Veazey, in contacting molten magnesium or magnesium alloy with a reducible manganese compound which reacts with such metal to liberate manganese metal in condition for direct alloying therewith. While 15 the manganese may be present in the ternary alloys in amounts of from 0.1 to 3.0 per cent or more, I normally prefer to keep the manganese content within the range of 0.5 to 1.5 per cent. Zinc, on the other hand, may be 20 present in amount from 0.5 to 16.0 per cent, although I normally prefer to keep within the range of 1.0 to 6.0 per cent. From my extensive work with this new alloy I have found 25 that where such ternary alloy contains approximately 95.6 per cent magnesium, 1.4 per cent manganese, and 3.0 per cent zinc, it is suitable for many uses, particularly where 30 corrosion resistance, as well as strength, is required.

35 Other modes of applying the principle of my invention may be employed instead of those explained, change being made as regards the composition herein disclosed, provided the ingredients stated by any of the following claims or the equivalent of such stated 40 ingredients be employed.

I therefore particularly point out and distinctly claim as my invention:—

1. As a new product, an alloy containing magnesium, manganese, and zinc, wherein the manganese is present in amount from 0.1 to 3.0 per cent, zinc in amount from 1.5 to 16.0 per cent, the balance being substantially magnesium.
2. As a new product, an alloy consisting of magnesium in amount in excess of 80 per cent and up to 99.4 per cent, manganese between 0.1 and 3.0 per cent, together with zinc in amount from 0.5 to 16.0 per cent.
3. As a new product, a ternary magnesium-manganese-zinc alloy wherein the magnesium is present in amount from 82.5 to 99 per cent, manganese from 0.5 to 1.5 per cent, and zinc from 0.5 to 16.0 per cent, the zinc content of the alloy exceeding the manganese.
4. As a new product, a ternary alloy of commercially pure magnesium, manganese, and zinc, wherein the magnesium is present in amount from approximately 88 to 99.5 per cent, manganese in amount from 0.1 to 2.0 per

cent, and zinc in amount from 0.5 to 10.0 per cent.

5. As a new product, an alloy consisting of magnesium in amount from approximately 92 to 98.5 per cent, manganese between 0.5 and 1.5 per cent, together with zinc in amount of 1.0 to 6.0 per cent.

6. As a new product, an alloy consisting of approximately 95.6 per cent magnesium, 1.4 per cent manganese, and 3.0 per cent zinc.

Signed by me this 13th day of November, 1930.

JOHN A. GANN.

80

85

90

95

100

105

110

115

120

125

130